

## UNITED STATES PATENT OFFICE

GUSTAV KOMAREK, OF CHICAGO, ILLINOIS, ASSIGNOR OF ONE-HALF TO KOMAREK-GREAVES & COMPANY, OF CHICAGO, ILLINOIS, A CORPORATION OF ILLINOIS, AND ONE-FOURTH TO GEORGE MACPHAIL AND ONE-FOURTH TO CHARLES CORYELL, BOTH OF BAY CITY, MICHIGAN.

## BRIQUETTE COMPOSITION AND PROCESS FOR MAKING BRIQUETTES

No Drawing.

Application filed July 25, 1929. Serial No. 381,080.

This invention relates to fuels and more particularly those having the form of briquettes adaptable for domestic and industrial usage.

It has long been known that petroleum coke from cracking stills or processes as well as from the paraffin departments of refineries possesses a high B. t. u. and is an excellent fuel. Large quantities are available and the problem has been to utilize the waste petroleum coke and thus make it a profitable by-product.

Attempts have been made to briquette this material in various ways but for the most part the briquettes have not been satisfactory, due to the crumbling, smokiness and the objectionable dirtiness which is a characteristic of the coke as it comes from the still or other source. The present invention has for its object to combine with petroleum coke, carbon coke in finely divided condition and in the form of fines or breeze and preferably fines or breeze from low temperature coke.

It has been found that coke fines and coke breeze, particularly that from low temperature coke, has an affinity for the high or excessive residual volatile and solid matter present in petroleum coke and such carbon coke being porous will absorb and diffuse sufficiently the free residuals.

It has, moreover, been found that the combination of petroleum coke and carbon coke following my invention can be so handled as to produce a briquette which will be practically smokeless and which will not crack but will hold and maintain its form during combustion.

The petroleum coke when combined with ordinary carbon coke in the form of fines or breeze, and particularly with breeze of low temperature carbon coke, will form a briquette, the rate of combustion of which is effectively controlled by reason of the presence of the low volatile carbon coke.

In this manner it is possible to combine the two materials in such proportion depending, of course, upon the analysis of the petroleum coke, that a briquette practically smokeless, slow burning and capable of holding its form without crumbling or forming

surface cracks during combustion is produced. This is attributable partly at least, to the fact that the high volatile matter present in the petroleum coke is diffused in the carbon coke, thus producing a retarded combustion.

In carrying out the invention, I take petroleum coke, which is the carbon and high molecular weight hydrocarbon solid substance formed during the pyrogenic decomposition of petroleum hydrocarbons in the well known cracking processes. Such coke, however, may be obtained from the paraffin department of a refinery and from other suitable sources.

This material has an approximate analysis as follows:

|                           |        |
|---------------------------|--------|
| Moisture, per cent        | 1.40   |
| Volatile matter, per cent | 12.03  |
| Fixed carbon, per cent    | 85.84  |
| Ash, per cent             | 0.84   |
| Sulfur, per cent          | 1.23   |
| B. t. u., per pound       | 15,293 |

The coke as it comes from the still or cracking plant is extremely dirty and objectionable because of the fine carbon soot it makes upon handling and of the oily stain it leaves wherever deposited. It usually consists of approximately seventy-five per cent (75%) dust and twenty-five per cent (25%) lump, the latter being about an inch in diameter and usually unstable.

The petroleum coke so obtained is crushed to fine condition and there is then admixed with it ordinary carbon coke, so that the two are thoroughly intermingled. By carbon coke is meant coke fines or coke breeze obtained in the production of ordinary coke from coal and I prefer to use the fines or breeze from low temperature coke.

The fines or breeze are porous and, as distinguished from the petroleum coke, have a low volatile content and are relatively slow burning.

Moreover, I have discovered that the coke fines or breeze, particularly from low temperature coke, possess an affinity for the free or excessive amount of volatile gases which are present in the petroleum coke and for

other residual and free solid matter also contained in the petroleum coke. These components of the petroleum coke are highly combustible and when the petroleum coke is 5 burned alone or in combination with materials not having the properties of the carbon coke employed in this invention, produce objectionable smoke and carbon stringers which I seek to eliminate.

10 When petroleum coke and the carbon coke in the form of breeze or fines are admixed, by reason of its affinity and porosity, the excessive amounts of residuals of volatile and solid matters from the petroleum coke, all 15 of which are highly combustible, are absorbed by the carbon coke and diffused through the mass.

In this manner the low volatile, slow burning carbon coke acts as a check upon the combustibility of the highly combustible free components of the petroleum coke. This, I have found, effectually solves the problem and permits the production of a smokeless briquette which will hold its form and which, 25 moreover, will be slow burning and completely combustible.

It will be clear that since the highly combustible free constituents of the petroleum coke are retained and diffused in the carbon 30 coke that the carbon coke will act as the controlling member for regulating the rate of combustion of the briquette.

The amount of carbon coke which is added will, of course, be proportional to the quantity of free residual volatile and solid constituents present in the petroleum coke.

For most purposes up to fifty per cent (50%) carbon coke will be satisfactory, but on the other hand, this amount may be increased and naturally decreased, since the analysis of petroleum coke from various stills will necessarily show a marked discrepancy.

The petroleum coke, therefore, is combined with the breeze or coke fines which are ordinarily a waste and which are preferably obtained from low temperature coking operations, and this carbon coke performs the several functions of absorbing the excess of 45 highly combustible residual matter contained in the petroleum coke as well as regulating the process and duration of combustion. The petroleum coke being highly combustible and the ordinary coke being relatively slow, naturally the rapidity of combustion is reduced and likewise this rate can be varied in accordance with the amount of carbon coke which is admixed.

The petroleum coke as removed from the 60 source of supply may be sufficiently moist and oily as to not require the use of a binder. In such cases, it is merely necessary to combine the breeze with the petroleum coke and briquette in the usual manner. Where, however, 65 there is not sufficient residual matter to allow

of immediate briquetting, a suitable binder is employed.

A large variety of such agents are available as for example hydrocarbon binders in the nature of asphalt or coal tar pitch in which case the briquette is usually coked at temperatures from 600 to 1500° F. This will produce a smokeless briquette, which holds its shape and does not crack or crumble while 70 burning.

Binders such as sulphite liquor, starch or inorganic binders may be used and the briquettes may then be used without further treatment or baked at temperatures from 350 to 600° F. or coked as above set forth.

The desirability of coking or baking, of course, will depend upon the nature of the briquette such as its moisture content or the binder employed and in many cases is not necessary or desirable.

In connection with heat treatment of the briquette, it is possible to produce a smokeless briquette from the petroleum coke and coke breeze or carbon coke by submitting the briquette after it has been formed to a moderate heat treatment of from 350 to 600° F. for the purpose of burning off any of the free combustibles upon the surface of the briquette. The purpose of the carbon coke, of course, is to absorb and diffuse all of the free residual combustibles of the carbon coke, but obviously there may be a small surface content in the briquette which, if given a moderate heating, can be effectively removed and the final briquette product will be substantially smokeless. As stated, the amount of coke fines or coke breeze will vary considerably, since if the residual matter in the petroleum coke is very high a much larger percentage of coke breeze would be used. The results and reaction, 100 however, are always the same.

Thus, with a briquette of dry petroleum coke, that is petroleum coke having a relatively low volatile and oily content, or heated to remove such content before being combined with coke breeze or coke fines, a highly improved combustion obtains which is unquestionably due to the strong attractions or affinity of the carbon coke for the volatile gases emitted from the petroleum coke.

It will be understood at this point that the petroleum coke may be in its original form as taken from the still or other source or it may be preliminarily treated to remove some of the volatile gases and oily component before being combined with the carbon coke. In either case, however, as explained, a more effective and cleaner combustion is obtained.

A practical test which I have made showed that briquettes from petroleum coke without the admixture of coke breeze would emit much smoke during combustion and an ordinary charge of twenty-five pounds fired in a stove would emit black smoke for thirty-five minutes and produce much objectionable soot

70

75

80

85

90

95

100

105

110

115

120

125

130

- in the form of long black stringers. The same petroleum coke briquette with forty per cent (40%) carbon coke in the form of breeze or fines from low temperature coke, and not heat treated, emits only light yellow smoke for twelve minutes and would produce no soot in the form of black stringers. The presence of the carbon coke brought about this very satisfactory result because the carbon coke absorbed a large amount of volatile gases present in the petroleum coke, thereby retarding combustion in that the highly inflammable volatiles were only released at a rate permitting complete combustion. At this point it should also be stated that when the petroleum coke and carbon coke after being briquetted, were given a moderate heat treatment, the burning was accomplished without any evidence of objectionable smoke or soot.
- It will be clear that the presence of the carbon coke acting to retard and control combustion of the briquette will serve an additional function, namely it will cause the briquette to hold its shape or form without cracking open or distorting due to swelling during combustion. Ordinarily, the briquettes are not preliminarily heat treated.
- In the practical use of the present invention when the briquettes are introduced into a domestic or industrial heating plant only the surface will ignite and as soon as it becomes heated no more smoke is emitted. This is due to the porosity of the breeze or fines which are distributed through the briquette and which have absorbed and act to store and maintain the excess volatile matter and free residuals present in the petroleum coke. This volatile content would otherwise distort and swell the briquette resulting in disruption of the surface crust and pass off as objectionable smoke. However, by storing or retaining them in the carbon coke and maintaining uncracked the surface crust, only the crust will burn and at the desired slow rate of combustion.
- It will be understood that I do not wish to be limited to the particular type of coke breeze or coke fines which are employed, but I find it preferable to use the breeze or fines obtained from low temperature coking.
- Moreover, it will be understood that the presence of the breeze or fines diffused through the mass of petroleum coke will act to absorb the volatile gases emitted by the petroleum coke and in this manner control the rate of combustion and cause the mass to retain its form without crumbling. At the same time, the B. t. u. of the petroleum coke is in no wise impaired and its value as a fuel becomes commercially realized.
- What I claim is:
1. A briquette comprising petroleum coke and a coke product of the destructive distillation of coal.
  2. A briquette comprising petroleum coke and a coke product obtained from low temperature destructive distillation of coal.
  3. A briquet comprising petroleum coke, and a porous comminuted coke product of the destructive distillation of coal, said coke product being present in sufficient amount to absorb and diffuse throughout the mass excess volatiles and combustible matter in the petroleum coke to control the rate of combustion.
  4. A briquet comprising petroleum coke having a relatively low content of volatiles and excess combustible matter, a coke product of the destructive distillation of coal, and a binder.
  5. The process of making a briquet comprising admixing petroleum coke and a coke product of the destructive distillation of coal, and heating to remove any free surface smoke forming substances.
- In testimony whereof I have hereunto set my hand.
- GUSTAV KOMAREK.